

Oct. 11, 1960

R. K. REMER

2,955,908

METHOD OF NEUTRALIZING SULPHUR-BEARING  
COMPOUNDS IN THE ATMOSPHERE

Filed June 3, 1957



FIG. 2



INVENTOR.

ROBERT K. REMER  
BY *Carl H. Lloyd*

EL771

# United States Patent Office

2,955,908

Patented Oct. 11, 1960

1

2,955,908

## METHOD OF NEUTRALIZING SULPHUR-BEARING COMPOUNDS IN THE ATMOSPHERE 5

Robert K. Remer, Elgin, Ill., assignor to Tribune Company, Chicago, Ill., a corporation of Illinois

Filed June 3, 1957, Ser. No. 663,063

11 Claims. (Cl. 21—2.5)

Generally, my invention relates to a method by means of which sulphur-bearing compounds present in the atmosphere may be neutralized. 15

More specifically, my invention relates to a method by means of which sulphur-bearing compounds, present in the atmosphere of an enclosure, may be neutralized.

It is a generally accepted fact that all air, especially that in the atmosphere surrounding industrial centers, contain certain sulphur compounds, such as hydrogen sulfide and sulphur dioxide. These sulphur compounds, even in the minute quantities commonly found in the normal atmosphere, react with metals, notably silver, and cause surface degradation, such as tarnishing.

Everyone is familiar with the problem of tarnishing on silver used in ornamental and artistic articles, and the labor and money necessarily expended to keep such articles lustrous. However, the tarnishing of silver presents a particular problem in the maintenance of electrical apparatus in which silver is employed in electrical conductors or contacts.

In many industrial situations where electrical conductivity and resistance is of a highly critical nature, such as in radio and television transmitting stations, silver is employed in electrical conductors or contacts, since its electrical conductivity is great, and fluctuations in its conductive properties caused by temperature changes and other outside factors, is minimal, in comparison with other conductors. When silver begins to tarnish, the conductivity and resistance of the metal is caused to vary greatly, depending upon the amount of tarnish.

Heretofore, the only method of combating the tarnishing of silver in such installations has been frequent polishing, which, particularly in cases where a large amount of silver is employed, is virtually a never-ending task.

Since sulphur-bearing compounds contained in the atmosphere are the primary cause of silver tarnishing, it is the premise of my invention that the neutralization of such compounds would reduce substantially the amount of labor and money expended in keeping silver tarnish-free.

Although the tarnishing of silver is, perhaps, the most readily apparent effect of sulphur-bearing compounds in the atmosphere, it should also be understood that many other undesired effects are caused by such compounds.

The main object of my invention is to provide a method by means of which sulphur-bearing compounds in the atmosphere may be neutralized.

Another object of my invention is to provide a method by means of which sulphur-bearing compounds may be neutralized and removed from a controlled current of air.

Still another object of my invention is to provide a self-regenerating method for the neutralization and removal of sulphur-bearing compounds from the air.

These and other objects and advantages of this invention will be apparent from the following description, taken in connection with the accompanying drawings, in which:

Fig. 1 is a diagrammatic view, partially broken away,

2

of a blower used in one method of practicing my invention; and

Fig. 2 is a view of a vaporizer which may be used in another method of practicing the invention.

In Fig. 1 I have shown a blower 10 of conventional construction (except as hereinafter described) for transmitting outside air into an enclosed area in which the apparatus to be protected is located. An intake portion 11 of the blower extends beyond an outside wall 12, and a fan, shown in outline at 13 directs the air through a conduit 14 which extends through a wall 15 of the enclosed area, indicated at 16. This area may be a machinery room or compartment in which I have shown diagrammatically a panel board or other mounting 17 for an electrical apparatus. The outlet of the conduit 14 is provided with a filter 18 held in place by a bracket 19. The filter 18 provides a means by which the sulphur-bearing compounds are neutralized and removed from the air conducted through said blower.

20 The filter may be fabricated from fibers of cotton, wool, silk, nylon, glass, Dacron, or regenerated cellulose. The base material thereof is impregnated with a mixture of chemicals which, upon contacting sulphur-bearing particles in the air which is to be blown therethrough, neutralize such particles and cause them to be retained in the filter. A combination of chemical compounds which I have discovered from experimentation to be well-suited for impregnating the fabric in order to impart such qualities thereto is a mixture of zinc acetate, a glycol, 25 acetic acid, and hydrazine sulphate. The interaction of these chemicals causes the filter to be regenerated in a manner hereinafter described.

25 The specific function of the zinc acetate in the filter is to act as a reactant with the sulphur-bearing compounds contained in the air. Sulphur compounds have a great affinity for zinc acetate, and when they come in contact with such a compound, they tend to join therewith in such manner as to be suspended within its molecular structure.

30 The glycol acts as a humectant, collecting water vapor from the air and causing the body of the filter to be damp at all times. I have found from experimentation that a filter which is slightly dampened is substantially more efficient than a dry filter.

35 The acetic acid tends to maintain the acidity of the fabric, which, during the course of operation of filtering the sulphur compounds from the air, would otherwise tend to become slightly alkaline.

40 The hydrazine sulphate is used as a catalyst. As the sulphur-bearing compounds contact the zinc acetate, zinc sulphide is formed. The hydrazine sulphate causes such zinc sulphide to reduce itself into two less complex chemical compounds, zinc acetate and an irreducible sulphur radical. The zinc acetate resulting from such reduction continues to attract sulphur-bearing compounds, 45 and the sulphur radical is suspended within the body of the filter. The sulphur radical being a group of atoms occurs in the molecules of sulphur compounds and remains unchanged in the filter until regeneration of the filter occurs.

50 As will be understood, the above described chemical reaction effects a continuing regeneration of the zinc acetate in the filter and causes the filter to be extremely long-lived.

55 The following has been found to be a suitable formulation of the above-mentioned chemicals for impregnating the body of the filter when this method of practicing the invention is employed:

|                                        | Parts |
|----------------------------------------|-------|
| Zinc acetate                           | 20    |
| Polyethylene glycol                    | 10-20 |
| Acetic acid of a strength of about 56% | .05   |
| Hydrazine sulphate                     | .05   |

Another way in which the invention may be practiced is to incorporate a zinc acetate compound in a candle and burn the candle in the enclosure in which the equipment or articles to be protected against tarnishing are located. This method would be practical in small enclosures in which the amount of atmosphere to be treated is relatively small. An example of a formulation which might be used in making such a candle is the following:

|                     | Parts |
|---------------------|-------|
| Sodium stearate     | 8     |
| Isopropyl myristate | 10    |
| Glycerine           | 6     |
| Alcohol             | 65    |
| Zinc acetate        | 6-20  |

A compound made from this formulation may be placed in a rectifier and molded into the customary form of a candle. The sodium stearate and isopropyl myristate react together to form a wax which constitutes the body of the candle. The glycerine and alcohol tend to dissolve, in part, the zinc acetate. Since both the glycol and the alcohol are highly volatile compounds, which are released when the candle burns, and since they contain portions of the zinc acetate which have been dissolved therein, they act as carriers to conduct the zinc acetate into the atmosphere to neutralize the sulphur-bearing particles therein.

The candle may be placed in the usual type of holder having a socket to receive the end of the candle, and the customary type of wick may be used.

Another formulation which is suitable for making such a candle is:

|                   | Parts |
|-------------------|-------|
| Sodium stearate   | 8     |
| Sorbitol          | 8     |
| Zinc acetate      | 8     |
| Isopropyl alcohol | 75    |

In this formulation, the sodium stearate would form the waxy body of the candle. The sorbitol and isopropyl alcohol would act to dissolve the zinc acetate. Since both of these compounds are highly volatile, they would cause the acetate to be conducted into the atmosphere in the manner above described.

Yet another method of removing sulphur-bearing compounds from the atmosphere of an enclosure might be the vaporization of a specially prepared chemical formula such as the following:

|                         | Parts |
|-------------------------|-------|
| Soap flakes             | 10    |
| Ammonia of 28% strength | 3     |
| Alcohol                 | 75    |
| Zinc acetate            | 20    |
| Mannitol                | 20    |

Such a formulation may be placed in a vaporizer indicated generally by the numeral 21 in Fig. 2 of the drawings. The soap flakes and the ammonia in this formulation combine to form a wax-like substance, a block or body 22 of which may be placed in water or other suitable liquid 23 in the vaporizer. Heat is then applied to the vaporizer as by a flame. The alcohol and mannitol tend to dissolve the zinc acetate. Since the alcohol and mannitol are highly volatile and such volatility is greatly increased by the application of heat to such a composition, the zinc acetate is conducted into the atmosphere of the enclosure to neutralize the sulphur-bearing compounds therein.

While several preferred procedures for practicing my invention have been described herein, it will be understood that modifications may be made therein without departing from the spirit and scope of the invention, and the specific disclosures herein contained should therefore be regarded as illustrative only.

I claim:

1. A method of neutralizing sulphur-bearing compounds in the atmosphere of an enclosure containing electrical installations employing silver conductors and the like, comprising dispersing zinc acetate into the atmosphere within said enclosure.
2. A method of neutralizing sulphur-bearing compounds in the atmosphere of an enclosure containing metal objects which are adversely affected by such compounds, comprising dispersing a volatile substance containing zinc acetate into the atmosphere within said enclosure.
3. A regenerative method of neutralizing sulphur-bearing compounds in the atmosphere of an enclosure containing metal objects which are adversely affected by such compounds, comprising conducting a stream of air containing such sulphur-bearing compounds into said enclosure through a mixture of zinc acetate, a glycol, acetic acid and hydrazine sulphate.
4. A regenerative method of neutralizing sulphur-bearing compounds in the atmosphere of an enclosure containing metal objects which are adversely affected by such compounds, comprising conducting a stream of air containing such sulphur-bearing compounds into said enclosure through a mixture of zinc acetate, a glycol, acetic acid and a catalyst adapted to reduce the sulphur-bearing compounds into zinc acetate and a sulphur radical.
5. A method of neutralizing sulphur-bearing compounds in the atmosphere of an enclosure containing metal objects which are adversely affected by such compounds, comprising releasing a volatile substance in which zinc acetate is partially dissolved into the atmosphere of the enclosure.
6. A method of neutralizing sulphur-bearing compounds in the atmosphere of an enclosure containing metal objects which are adversely affected by such compounds, comprising dissolving zinc acetate in a composition which will arrest the volatility thereof under normal temperatures but will release the same when heated, and applying heat to said composition, thereby liberating the volatile substance therefrom and causing the zinc acetate to be dispersed in the atmosphere within the enclosure.
7. A method of neutralizing sulphur-bearing compounds in the atmosphere of an enclosure containing metal objects which are adversely affected by such compounds, comprising dissolving zinc acetate in a composition comprising soap flakes, ammonia, alcohol and mannitol, which composition is stable within a normal range of temperature but will release the same when heated, and applying heat to said composition, thereby liberating the volatile substance contained therein and causing the zinc acetate to be dispersed into the atmosphere within the enclosure.
8. A method of neutralizing sulphur-bearing compounds in the atmosphere of an enclosure containing metal objects which are adversely affected by such compounds, comprising dissolving zinc acetate in a volatile substance, incorporating such volatile substance in a candle, and burning such candle within the enclosure, thereby dispersing the zinc acetate contained therein into the atmosphere within such enclosure.
9. A method of neutralizing a sulphur-bearing compound in the atmosphere of an enclosure containing metal objects which are adversely affected by such compound, comprising burning in such enclosure a candle made from a formula including sodium stearate, isopropyl myristate, glycerine, alcohol and zinc acetate, thereby causing dispersion of the zinc acetate in the atmosphere within the enclosure to neutralize said sulphur-bearing compound.
10. A method of neutralizing a sulphur-bearing compound in the atmosphere of an enclosure containing metal objects which are adversely affected by such compound, comprising burning in such enclosure a candle made from a formula including sodium stearate, sorbitol, iso-

propyl alcohol and zinc acetate, thereby causing dispersion of the zinc acetate in the atmosphere within the enclosure to neutralize said sulphur-bearing compound.

11. A method of neutralizing sulphur-bearing compounds in the atmosphere of an enclosure containing metal objects which are adversely affected by such compounds, comprising conducting a stream of air containing methyldichlorosilane, benzol, water and zinc acetate.

## References Cited in the file of this patent

## UNITED STATES PATENTS

|           |          |               |
|-----------|----------|---------------|
| 1,628,610 | Osborne  | May 10, 1927  |
| 2,323,804 | Driscoll | July 6, 1943  |
| 2,516,340 | Pirchio  | July 25, 1950 |
| 2,701,238 | Renold   | Feb. 1, 1955  |